

## UNITED STATES PATENT OFFICE

2,074,338

## LUBRICATING OILS

Bert H. Lincoln, and Alfred Henriksen, Ponca City, Okla., assignors, by mesne assignments, to The Lubri-Zol Development Corporation, Cleveland, Ohio, a corporation of Delaware

No Drawing. Application May 12, 1932, Serial No. 610,988

12 Claims. (Cl. 87—9)

This invention relates to an improvement in lubricating oils, and more particularly to an oil of increased lubricity.

Under conditions of boundary lubrication the viscosity of the lubricant plays only a minor part in lubrication. With slow speeds and heavy loads contributing to boundary lubrication, the lubricant to be efficient must have a high degree of oiliness or unctuousness and must have a high film strength. The very best mineral oils are, as a rule, very deficient in oiliness character and film strength, resulting in considerable wear, low efficiency, and at times seizure of metals in machines lubricated with mineral oils only. For these particular duties lubricating engineers have used animal and vegetable oils with some success, but the changes occurring in the animal and vegetable oils during use have made them very unsatisfactory for general use, as well as uneconomical due to the expense of the fatty oils and the quantities required.

Mineral oils having low film strength allow seizure of the rubbing surfaces when, for one reason or another, pressures are increased or the rubbing speed is slow.

Objects of this invention are to provide a lubricant with high oiliness character and high film strength without introducing the objectionable features of lubricating oil sludging, gumming, rancid odor and perceptible corrosion. The application of this invention realizes these objects very economically.

It has been found that commercial stearic acid as found on the market and other saturated fatty acids, when blended with mineral lubricating oil, will greatly reduce the coefficient of friction. As an example, a good grade mineral oil had a coefficient of friction of 0.135 to 0.140 when tested on the Herschel friction testing machine with a 40% lead disc. (The Herschel friction testing machine is a development by Dr. W. H. Herschel of the U. S. Bureau of Standards.) When 0.5% commercial stearic acid was added to the above mineral oil, it had a coefficient of friction of only 0.055. Thus, by adding a very small amount of stearic acid, the coefficient of friction was only 39 to 41% as great as with the original oil.

The melting point of commercial stearic acid is around 100–170° F., depending upon the impurities present in the commercial acid. (These impurities do not affect the value of this invention, it being found that any of the commercial stearic acids are suitable.) Stearic acid is completely soluble in mineral oil at high temperatures, but due to its high melting point, the stearic acid starts solidifying as the temperature goes below say 100° F. and at low temperatures, say around 15 to 30° F., will in time settle out of the solution. This is a common characteristic of the saturated fatty acids of high melting point, which

requires their use in warm weather and prohibits storage and use of lubricants prepared in this manner during cold weather. With this knowledge, the use of saturated fatty acids in mineral oil may be economically and efficiently applied in a number of places.

It has been found, however, that the solubility and film strength of fatty acids can be greatly improved by halogenation. The halogenated fatty acids will remain in solution over long time storage during cold weather and will not cause sludging of the lubricant, gumming or other objectionable features. Addition of halogen to the fatty acid molecule lowers the melting point and accomplishes this very beneficial result and makes them available for economical use under any kind of temperature conditions.

As an example of this, ordinary commercial stearic acid (a saturated acid) with a melting point around 120–140° F. was chlorinated direct with chlorine until the chlorinated product had a melting point of 62° F. Excess free chlorine and hydrochloric acid are removed by any of the ordinary means and the chlorinated product added to mineral oil lubricants in small quantities. The poorer the quality of the original lubricating oil the more the chlorinated acid required. The Herschel friction testing machine was used to determine the increased oiliness. The original mineral oil showed a coefficient of friction of 0.135 to 0.140%. Chlorinated stearic acid was added in quantities of from .05% to .5% with the following results:

| Amt. of chlor. stearic acid added to mineral lubricant | Coefficient of friction on Herschel friction machine |
|--------------------------------------------------------|------------------------------------------------------|
| Original mineral lubricant                             | 0.135 to 0.140                                       |
| .05%                                                   | 0.072 to 0.077                                       |
| .1%                                                    | 0.070 to 0.075                                       |
| .25%                                                   | 0.070 to 0.075                                       |
| .50%                                                   | 0.070 to 0.075                                       |

Another sample of commercial stearic acid was chlorinated until the chlor acid had a melting point of 9° F. This product was added to the same mineral oil with the following results:

| Amt. of chlor. stearic acid added to mineral lubricant | Coefficient of friction on Herschel machine |
|--------------------------------------------------------|---------------------------------------------|
| Original mineral lubricant                             | 0.135 to 0.140                              |
| .05%                                                   | 0.075 to 0.080                              |
| .10%                                                   | 0.075 to 0.080                              |
| .25%                                                   | 0.075 to 0.080                              |
| .5%                                                    | 0.115 to 0.120                              |

Both of the above examples clearly show that the maximum reduction in coefficient of friction

is obtained with small quantities of the chlor fatty acid. In the case of the fatty acid chlorinated to 9° F. melting point, the coefficient of friction increased when the amount of acid added reached 0.5%. As previously stated, with a poorer quality original mineral oil as much as 2% or more acid may be required to get the same reduction in coefficient of friction.

Commercial oleic acid representing the field 10 of unsaturated fatty acids was chlorinated to partial saturation and sufficient chlorine added to prevent acid sludging or polymerization of the unsaturated acid. This product, when added to a mineral lubricant having an original coefficient 15 of friction of 0.135 to 0.140, gave the following result.

|    | Chloroleic acid added        | Coefficient of friction<br>Herschel machine |
|----|------------------------------|---------------------------------------------|
| 20 | 0.5%<br>Original mineral oil | 0.065 to 0.070<br>0.135 to 0.140            |

It has been found that unsaturated free fatty acids will reduce the coefficient of friction when used in small quantities. For example, 0.5% of oleic acid in a mineral oil having an original coefficient of friction of 0.135 to 0.140 gave a product with a coefficient of friction of 0.055 to 0.060.

30 To determine the film strength of lubricants under high pressure, two testing machines have been developed. One is called the Mougey machine and was perfected by Dr. H. G. Mougey of the General Motors Corporation and has been described by the inventor in various literature. The other machine is known as the Timken machine and was developed by the Timken Roller Bearing Company, which has also been described in the literature. The primary object of these 40 machines is to give very high pressure per unit area of rubbing surfaces under conditions resembling those found in commercial use but probably a little more severe. The lubricant is placed between the friction surfaces and used 45 with increasing pressure or load at the friction point until seizure of the metal surfaces occurs. With the Mougey machine the pressure or load may be held constant and determine the time required for seizure of the metal surfaces. By the 50 use of these machines it is easy to compare the film strength of two oils.

Using the Mougey machine a good grade mineral oil allowed seizure of the friction surfaces in 30 minutes with a load of 2000# per square inch. 55 Using another sample of the same mineral oil blended with 0.5% of chlorstearic acid of 9° F. melting point and operating the Mougey machine at 2000 pounds per square inch pressure, there were no signs of seizure after a period of 45 minutes, proving a decided superiority of film strength in the lubricant blended with chlorstearic acid. With higher pressures, larger quantities of the chlorstearic acid should be used—as much as 5% or more being required.

65 Using the timken machine with the original lubricant seizure of metal surfaces occurred when 18.2# weights had been added, which represent a pressure of approximately 10,500 pounds per square inch. To a sample of this same lubricant 70 0.25% of chlorstearic acid of 9° F. cold test was added, and when this blended lubricant was used in the Timken machine seizure did not occur until a 32.2# weight had been added representing a pressure of approximately 19,000 pounds per 75 square inch.

Repeating the test on the Timken machine with the same original lubricant containing 0.5% of chlorstearic acid of 9° F. melting point, metal seizure did not occur until 38.0 pound weights had been added, which represents a pressure of approximately 22,000 pounds per square inch. Thus, by adding 0.5% of the product of this invention to a high quality lubricant, its film strength is more than doubled.

The above tests clearly demonstrate the economy and efficiency of the process and show that by this invention it is possible to prepare a lubricant for practically any duty by either varying the percentage of product blended and/or varying the degree of halogenation of the product to be 15 blended.

It has also been found that lubricants prepared by this invention do not lose their oiliness characteristics when diluted with small amounts of unburned motor fuel, making this type of lubricant of unusual value in actual commercial lubrication conditions.

The addition of halogenated fatty acids in the manner of our invention reduces sludging or polymerization in the oil. For example, using the 25 Tidewater oxidation test, which consists in determining the amount of sludge formed in an oil after heating for seven hours at 392° F., the following results were obtained:

300 reduced oil + 0.5% oleic acid gave a sludging number of 91.6 while the same oil with 0.5% of halogenated oleic acid gave a sludging number of 72.4 or a reduction in sludging number of 19.2.

Having thus described our invention, what we 35 claim is:

1. A lubricant comprising in combination a mineral oil and a small percentage of a halogenated higher fatty acid of the aliphatic series.

2. A lubricant comprising in combination a mineral oil and a small percentage of a chlorinated higher fatty acid of the aliphatic series.

3. A lubricant comprising in combination a mineral oil and a small percentage of halogenated stearic acid.

4. A lubricant comprising in combination a mineral oil and a small percentage of halogenated oleic acid.

5. A lubricant comprising in combination a mineral oil and a small percentage of chlorinated stearic acid.

6. A lubricant comprising in combination a mineral oil and a small percentage of chlorinated oleic acid.

7. A lubricant comprising in combination a mineral oil and a small percentage of a halogenated unsaturated fatty acid.

8. A lubricant comprising in combination a mineral oil and a small percentage of a halogenated saturated fatty acid.

9. A lubricant comprising in combination a mineral oil and a small percentage of a halogenated acyclic, monocarboxylic acid.

10. A lubricant comprising in combination a mineral oil and a small percentage of a chlorinated acyclic monocarboxylic acid.

11. A lubricant comprising in combination a mineral oil and a small percentage of a halogenated acid of the acrylic series.

12. A lubricant comprising in combination a mineral oil and a small percentage of a chlorinated acid of the acrylic series.